

No. 861,224.

PATENTED JULY 23, 1907.

E. F. PRICE.

PROCESS OF PRODUCING FERROSILICON.

APPLICATION FILED NOV. 14, 1905.



Witnesses:

*Ed. E. Gault*  
*J. B. Hill*

Inventor:

*Edgar F. Price*  
*by Gurnee & Townsend,*  
*Atty's.*

# UNITED STATES PATENT OFFICE.

EDGAR F. PRICE, OF NIAGARA FALLS, NEW YORK.

## PROCESS OF PRODUCING FERROSILICON.

No. 861,224.

Specification of Letters Patent.

Patented July 23, 1907.

Original application filed August 31, 1904, Serial No. 222,891. Divided and this application filed November 14, 1905.  
Serial No. 287,346.

To all whom it may concern:

Be it known that I, EDGAR F. PRICE, a citizen of the United States, residing at Niagara Falls, in the county of Niagara and State of New York, have invented certain new and useful Improvements in Processes of Producing Ferrosilicon, of which the following is a specification.

In my application 222,891, filed August 31, 1904, which matured into Patent 790,391 of May 23, 1905, I described and claimed a process of smelting an electrically-conductive charge, specifically one containing chromite for the production of ferrochromium. The present application is a division of said earlier one and the claims are specifically directed to the production of ferrosilicon.

A suitable electric furnace is shown in the accompanying drawing, in which the figure is a vertical axial section through the tap-holes, with the electrodes in elevation.

20 The furnace comprises a body 1 of firebrick or masonry, with a refractory lining 2 of magnesite, siloxicon or carbon. Lateral tap-holes 3, 4 for slag and metal, respectively, extend from the lower part of the furnace chamber. The electrodes 5, 6 of opposite polarity, shown as carbon rods, depend into the furnace. In employing this furnace to carry out the process, an arc is established between the electrodes or each electrode and the carbon lining 2, if used, and a small amount of the charge is fed into the bottom of the furnace. 30 The charge may consist of a mixture of silica, iron or iron ore and coke, in which the ingredients are in such proportion as to make it a partial conductor when hot, or which contains pieces of iron or magnetite and coke which tend to shunt the current. The furnace is then gradually filled until, in its normal working condition, the electrodes are embedded in the charge 7, as illustrated. The minimum voltage is applied to the electrodes, to largely prevent the electric current from shunting through the charge. As the iron 40 and silicon are reduced, a layer 8 of the molten alloy collects in the bottom of the furnace and may be removed from time to time through the tap-hole 4. If the charge contains impurities, a layer of slag may accumulate upon the metal, and is removed through the tap-hole 3.

It will be seen that the deep body of the charge 7 surrounding the electrodes effectively retains the heat within the furnace, both increasing the production of metal and maintaining the contents in a molten condition without especial attention. The use of this deep

body is made possible by and necessitates the employment of a minimum electromotive force, since the voltage usually employed in furnaces of this character would cause excessive waste of current by shunting or short circuiting through the charge, if no current-regulator were employed, a commercially-impracticable mode of procedure; or would lift the electrodes partially out of the charge if controlled by a constant-current regulator, thus raising the zone of maximum temperature to the upper part of the furnace and causing excessive heat losses by radiation from the charge, excessive oxidation of the hot exposed surfaces of the electrodes, and loss of a portion of the finely-divided charge by the gases blowing violently out from the zone of reduction. The furnace is operated continuously, 55 the metal and any slag being drawn off and fresh materials added as required. The hot surfaces of the electrodes and furnace lining are therefore never exposed to the oxidizing and cooling action of the atmosphere. 60

While the furnace shown employs two depending 70 electrodes of opposite polarity, it is obvious that the process may be carried out by the use of a furnace in which the hearth surface is one electrode, the arc being sprung between the hearth and a single depending electrode.

I claim:

1. The process of producing ferrosilicon by smelting an electrically-conductive charge of a silicon compound, carbon and a source of iron, which consists in establishing an electric arc within the charge, surrounding the zone of reduction and protecting the electrodes from the oxidizing and cooling effect of the atmosphere by a considerable body of the charge, and maintaining between the electrodes the minimum potential difference requisite to effect reduction, thereby substantially preventing loss of electric current by leakage through the charge and heat radiation, as set forth.

2. The process of producing ferrosilicon by smelting an electrically-conductive charge of a silicon compound, carbon and a source of iron, which consists in establishing an electric arc within the charge, surrounding the zone of reduction and protecting the electrodes from the oxidizing and cooling effect of the atmosphere by a considerable body of the charge, maintaining between the electrodes the minimum potential difference requisite to effect reduction, thereby substantially preventing loss of electric current by leakage through the charge, tapping the product from the furnace, and supplying the charge-mixture as required, as set forth.

In testimony whereof, I affix my signature in presence of 100 two witnesses.

EDGAR F. PRICE.

Witnesses:

G. E. COX,  
D. BURGESS.